

# United States Patent Office

2,927,067

Patented Mar. 1, 1960

1

2,927,067

## ELECTROREFINING OF ZIRCONIUM

William W. Gullett, College Park, Md., assignor to Chicago Development Corporation, Riverdale, Md., a corporation of Delaware

No Drawing. Application October 17, 1957  
Serial No. 690,611

1 Claim. (Cl. 204—64)

This invention relates to electrorefining of zirconium. It relates particularly to refining in electrolytes composed of fused alkalinous metal chlorides, that is, alkali or alkaline earth metal chlorides or mixtures of them, having dissolved therein zirconium chlorides. I have found that zirconium oxide which is formed by the solution of crude zirconium containing oxygen is not substantially soluble in such electrolytes and hence the cathode deposit is not contaminated by oxygen from the anode.

I have found that the electrolytic bath must contain at least one lower chloride of zirconium in solution in the bath. The bath is defined by a series of equilibria as follows:



and also by disproportionation equilibria



I have found that Reaction 5 may be practically disregarded and that the bath to be useful for refining must correspond primarily to Reaction 2 and that Reaction 4 must be prevented from running from right to left by which the bath would be converted into finely divided Zr and  $\text{ZrCl}_4$  which would volatilize.

This is accomplished by a low concentration of  $\text{ZrCl}_2$ , a low temperature and increased pressure.

I have found that at atmospheric pressure, a concentration of dissolved zirconium in a lower valence state of 1-2% is preferable and that a suitable alkalinous metal bath is composed of 65%  $\text{SrCl}_2$  and 35% NaCl. This electrolyte melts at a comparatively low temperature and does not break into two layers.

It is necessary in carrying out the refining to avoid increased local concentrations of dissolved lower chlorides of zirconium. This is preferably accomplished by anodic solution from a small surface which is vibrated to prevent concentration polarization.

In another embodiment of the invention, Reaction 4 is forced from right to left by pressure and a large surface of the Zr to be refined, and a cathode is placed at minimum distance from the dissolving Zr so that the reaction cycle of solution diffusion and disproportionation is reduced by deposition on the cathode before the concentration for disproportionation takes place.

The electrolytic bath for my invention may be made in a number of ways. One of the preferred ways is heating Zr,  $\text{PbCl}_2$ ,  $\text{SrCl}_2$  and NaCl in a closed tube to about 800° C. The preferred proportions are 1 mole of Zr to 1 of  $\text{PbCl}_2$ , with the eutectic proportions of  $\text{SrCl}_2$  and NaCl so as to obtain a 5% concentration of Zr in the electrolyte. Such an electrolyte will contain about 2% Zr as lower chlorides.

This electrolyte may be used at low temperatures and relatively high pressures, or it may be heated to 800° C. at atmospheric pressure with vibrated Zr strips in the

2

bath to partly reduce  $\text{ZrCl}_4$  present and in part to distill it off.

In another procedure for preparing an electrolytic bath for my invention, I add  $\text{ZrCl}_4$  and sodium in amounts corresponding to  $\text{ZrCl}_2$  in small increments to  $\text{SrCl}_2$  in a pot heated to 600° C. provided with a condenser which can be cleared by rodding. The product of this operation was a mixture of  $\text{ZrCl}_2$ ,  $\text{ZrCl}_3$ ,  $\text{ZrCl}_4$ , NaCl and sodium.

10 This mass could be melted at 750° C. under 25 lbs. argon pressure and used as an electrolytic bath in which the zirconium in it served as a disperse anode, the pot which carried the anodic current being very close to the cathode which was preferably preformed to provide a layer of salt with dispersed fine crystals.

Having now described my invention in its most general terms, I will illustrate it by examples.

### Example I

20 In this example, I take 900 grams of Zr scrap and mix it with 2780 grams of  $\text{PbCl}_2$  and 18,000 grams of an eutectic mixture of  $\text{SrCl}_2$  and NaCl and seal in a heavy iron tube. I heat to 800° C. for 2 hours, I open the iron tube and recover about 2080 grams of lead in a button and 15,020 grams of fused salt containing chlorides of zirconium and a little lead chloride. I melt this mixture in an iron pot 2" in diameter in an argon atmosphere at 1000° C., add 100 grams  $\text{ZrO}_2$  and vibrate a zirconium strip in it for 15 minutes. I then cool 25 to 750° C. and allow the solids to settle.

I now place zirconium scrap analyzing .370%  $\text{O}_2$  in a hollow iron anode chamber 1 inch in diameter with small openings below the bath, place this at the center of the pot and vibrate this to provide anodic solution.

30 I now place the removable iron liner in the pot as cathode and electrolyze at 10 amperes for 10 hours. I remove the cathode by raising into an argon atmosphere and on cooling, I remove the coarse crystalline product and wash with 2% HCl. 100 grams of zirconium was recovered, which when melted in argon had a Brinell hardness of 80.

The structure of the cathode deposit was a zirconium plate on the cathode, a thin layer of salt with fine zirconium crystals and an outer layer of crystal intergrowths constituting more than 90% of the cathode product.

### Example II

45 In this example, I take 2300 grams  $\text{ZrCl}_4$  and 920 grams of sodium and add them in small increments to a pot at 700° C. provided with a condenser. I rod the condenser frequently to clear it of sublimed  $\text{ZrCl}_4$  which falls in the reaction pot. I place in the bottom of the pot at the start 3000 grams  $\text{SrCl}_2$ . When reaction is complete, I cool the mass in an argon atmosphere, and break it out of the pot. I place this mass in a heavy walled Inconel tube 2" in diameter and provided with a centrally disposed iron rod cathode insulated from the tube. A cover is provided to withstand 50 lbs. pressure having a packing gland and lock for the cathode, an argon inlet and a lock for adding comminuted crude zirconium. The cathode 50 can be lifted into the cool upper portion of the tube and removed and replaced through a suitable lock.

55 When the lower portion of the tube has been heated to 750° C. under 50 lbs. pressure, 10 amperes is passed for 10 hours and then the cathode lifted, and removed from the cell. Approximately 100 grams of coarse crystalline Zr is recovered from the cathode.

60 Analyses of the crude zirconium and the recovered crystals was as follows:

|          | Percent oxygen |
|----------|----------------|
| Crude Zr | .3             |
| Product  | .005           |

The structure of the cathode deposit in this example was like that described for Example 1.

What is claimed is:

The process of electrorefining crude zirconium which consists in making it a disperse anode in an electrolyte at 700-900° C. under a pressure above atmospheric in a fused bath of the reaction product of one mole zirconium tetrachloride with approximately two moles of sodium in strontium chloride at 500-700° C., having an inert cathode closely spaced to said disperse anode and passing a unidirectional current from said anode to said cathode whereby to form pure coarse crystalline zirconium on the cathode.

References Cited in the file of this patent

UNITED STATES PATENTS

|           |                |               |
|-----------|----------------|---------------|
| 2,061,146 | Ferrand        | Nov. 17, 1936 |
| 2,734,856 | Schultz et al. | Feb. 14, 1956 |
| 2,746,732 | Guillette      | May 22, 1956  |
| 2,782,156 | Raynes         | Feb. 19, 1957 |
| 2,785,066 | Dean           | Mar. 12, 1957 |
| 2,817,630 | Dean           | Dec. 24, 1957 |
| 2,817,631 | Gullett        | Dec. 24, 1957 |
| 2,821,506 | Wainer         | Jan. 28, 1958 |
| 2,838,393 | Dean           | June 10, 1958 |
| 2,845,386 | Olson          | July 29, 1958 |

OTHER REFERENCES

15 "Electrolytic Titanium," Chicago Development Corp.